

Dec. 31, 1963

J. S. KOUVEL

3,116,182

MAGNETS

Filed May 29, 1961

Fig. 1.



Fig. 2.



Fig. 3.



Fig. 4.



Inventor:  
James S. Kouvel,

by Richard L. Green  
His Attorney.

1

3,116,182

## MAGNETS

James S. Kouvel, Albany, N.Y., assignor to General Electric Company, a corporation of New York  
Filed May 29, 1961, Ser. No. 113,411  
4 Claims. (Cl. 148—31.57)

This invention relates to magnets and more particularly to magnets having one easy direction of magnetization and to a method for producing such magnets.

Previously known magnetic materials have been most readily magnetized along one or more axes and have been equally readily magnetizable in either direction along each axis. The magnetic properties of these materials have been measured and evaluated by several methods, perhaps the best known being the graphical representation of the hysteresis loop obtained when a magnetic field is applied to the magnetic material in such a manner as to cyclically reverse polarity. Since magnetic properties have been symmetrically reversible, both quantitatively and qualitatively with respect to the axis of magnetization, the magnets have at least two stable positions in a strong magnetic field.

While existing magnetic materials have generally proven acceptable for use in most situations, the increasing use of electronic and electrical apparatus under unusual environmental conditions has resulted in a need for components having particular properties when subjected to such unusual conditions. For example, various parts of guidance or computer systems must be able to perform reliably at extreme temperatures. Development of these and other technological areas has resulted in recognition that a magnetic material having one easy direction of magnetization would be of value, particularly where this property could be utilized at low temperatures.

A principal object of this invention is to provide magnets having one easy direction of magnetization.

Another object of this invention is to provide an alloy magnet consisting essentially of manganese alloyed with a metal from the group of copper, silver and gold which has one easy direction of magnetization.

An additional object of this invention is to provide a process for producing magnets having one easy direction of magnetization.

Other objects and advantages of this invention will be in part obvious and in part explained by reference to the accompanying specification and drawings.

In the drawings:

FIGURE 1 shows a hysteresis loop illustrating the magnetic characteristics of the usual type permanent magnet;

FIGURE 2 shows a hysteresis loop illustrating the magnetic characteristics of a copper-manganese magnet made according to the present invention;

FIGURE 3 shows a hysteresis loop illustrating the magnetic characteristics of a silver-manganese magnet made according to the present invention; and

FIGURE 4 is a hysteresis loop illustrating the magnetic properties of a magnet constructed of the same alloy used for FIG. 2 but which was not subjected to a magnetic field during cooling.

Generally, this invention concerns permanent magnets and a process for producing permanent magnets having one easy direction of magnetization, which magnets comprise bodies containing from about 5 to 30 atomic percent manganese, balance substantially all a metal selected from the group consisting of copper, silver and gold. The process for producing these magnets generally comprises preparing a suitable alloy body and cooling the alloy body in a magnetic field to a tem-

2

perature sufficiently low to create the one easy direction of magnetization, generally 90° K. or less.

It has been mentioned previously that existing alloy magnets have at least two easy directions of magnetization and also have two equivalent stable positions in an applied magnetic field.

The hysteresis loop 10 characteristic of the usual type permanent magnets is shown in FIG. 1, in which the magnetizing field  $H$ , in oersteds, is the axis of the abscissa and the magnetization or  $M$ , in e.m.u. is the axis of the ordinate. As the field is increased from zero to higher values of  $H$  in what for convenience may be referred to as the positive direction, the magnetization ( $M$ ) of the material reaches a maximum value  $+M_{max}$  for a given field. If the field  $+H$  is removed, the value of the magnetization decreases along the demagnetization curve 11 to  $M_{R1}$ . If then a field  $-H$  of reverse polarity is applied, the magnetization of the material continues to decrease along curve 11 and crosses the  $H$  axis at the value  $H_{c1}$ , the magnetization finally reaching  $-M_{max}$  as the field is further increased in the negative direction. If the negative field is removed, the magnetization of the material correspondingly drops to  $M_{R2}$ , which is numerically equal to  $M_{R1}$ . Application of the positive field then causes the magnetization to move along the magnetization curve 12 and cross the  $H$  axis at the value  $+H_{c2}$ , which is numerically equal to  $H_{c1}$ . As the positive field is increased, the magnetization of the material rises to the value  $+M_{max}$ . The magnetization values  $M$  which were used in the present case in place of the flux density,  $B$ , to plot the hysteresis loops, are equal to the flux density ( $B$ ) minus the magnetizing field ( $H$ ), divided by  $4\pi$ , as indicated by the formula:

$$M = (B - H) / 4\pi$$

Alloys which can be used, as previously mentioned, to produce magnets having one easy direction of magnetization consist essentially of copper or silver or gold alloyed with from 5 to 30 atomic percent manganese. The copper-manganese alloys will generally contain from 5 to 30 atomic percent manganese, balance substantially all copper, whereas the silver and gold percentages will generally fall within the range of from 15 to 25 atomic percent, balance substantially all manganese.

FIGURE 2 of the drawings shows a hysteresis loop 15 which is characteristic of the magnets of the present invention. The composition of the magnet used to produce loop 15 was 24.1 atomic percent manganese, balance copper. Here the loop is shifted toward the negative direction of field, the material thus being more easily magnetized in the positive direction. The maximum fields  $-H_{max}$  and  $+H_{max}$  are quantitatively the same, about 10,000 oersteds, but the magnetization values  $M_{R1}$  and  $M_{R2}$  are both positive and the field strength  $H_{c1}$  and  $H_{c2}$  are both negative. It will be noted that the loop is extremely thin, so that the field and magnetization values are essentially the same, viz., 4,000 oersteds and 7.5 e.m.u., respectively. Since the two values for  $M_R$  have the same sign (and magnitude), the material in zero field is magnetized in the same direction, regardless of the direction of any field previously impressed on it.

Curve 16, FIGURE 3, illustrates the magnetic properties of a magnet having the composition 23.7 percent manganese, balance substantially all silver. Once again the magnetization values are both positive, about 7 e.m.u., and the field strengths both negative, about 3,750 oersteds.

Examples of several alloys which can be processed to develop the desired properties follow. Only one value is listed for  $M_R$  and  $H_c$ , since the magnetizations were both positive and about the same and the field strengths were both negative and about the same.

3  
Table I

| Alloy                    |                          |                          | +M <sub>R</sub><br>(e.m.u.) | -H <sub>c</sub><br>(oer.) | Approx.<br>Temp.<br>Where<br>Effect<br>Disappears,<br>°K. |
|--------------------------|--------------------------|--------------------------|-----------------------------|---------------------------|-----------------------------------------------------------|
| Mn,<br>Atomic<br>percent | Cu,<br>Atomic<br>percent | Ag,<br>Atomic<br>percent |                             |                           |                                                           |
| 5.5                      | 94.5                     | ----                     | 5                           | 150                       | 10                                                        |
| 8.9                      | 91.1                     | ----                     | 13                          | 200                       | 20                                                        |
| 14.0                     | 86.0                     | ----                     | 19                          | 350                       | 30                                                        |
| 18.9                     | 81.1                     | ----                     | 11                          | 1,700                     | 50                                                        |
| 24.1                     | 75.9                     | ----                     | 7                           | 4,000                     | 70                                                        |
| 28.6                     | 71.4                     | ----                     | 4                           | 11,000                    | 90                                                        |
| 11.9                     | ----                     | 88.1                     | 12                          | 200                       | 10                                                        |
| 15.9                     | ----                     | 84.1                     | 10                          | 900                       | 20                                                        |
| 20.0                     | ----                     | 80.0                     | 9                           | 1,900                     | 25                                                        |
| 23.7                     | ----                     | 76.3                     | 7                           | 3,400                     | 35                                                        |

Since the gold-manganese alloys exhibit hysteresis loops which cannot be characterized by single values of M<sub>R</sub> and H<sub>c</sub>, sample compositions of these alloys are set forth in Table II, together with their magnetic properties.

Table II

| Alloy                    |                          | M <sub>R1</sub><br>(e.m.u.) | M <sub>R2</sub><br>(e.m.u.) | H <sub>c1</sub><br>(oer.) | H <sub>c2</sub><br>(oer.) | Approx.<br>Temp.<br>Where<br>Effect<br>Disappears,<br>°K. |
|--------------------------|--------------------------|-----------------------------|-----------------------------|---------------------------|---------------------------|-----------------------------------------------------------|
| Mn,<br>Atomic<br>percent | Au,<br>Atomic<br>percent |                             |                             |                           |                           |                                                           |
| 15                       | 85                       | +72                         | -58                         | -850                      | +100                      | 10                                                        |
| 20                       | 80                       | +150                        | -135                        | -500                      | +150                      | 20                                                        |
| 23                       | 77                       | +1.6                        | +1.2                        | -1,000                    | -850                      | 60                                                        |

As has already been stated, the treatment to which the alloys must be subjected is important in achieving magnets having the magnetic properties evidenced by the shifted hysteresis loops. It is felt that both atomic and magnetic heterogeneity must exist to develop the one easy direction of magnetization, that is, some degree of disorder should exist to bring about the shifted hysteresis loop characteristic, although complete disorder is probably not essential as some residual order may exist in almost all systems.

As generally understood, a disordered solid solution alloy is one in which the atoms of the various constituent metals of an alloy are randomly distributed through the alloy lattice. Conversely, an ordered solid solution alloy is one in which the atoms of the different metals repeat in lattice position according to a definite pattern.

Broadly, the process involves preparing a magnet body of a suitable alloy such as one of those previously disclosed, quenching the body from an elevated temperature to retain some degree of atomic disorder and cooling the body in a magnetic field to below the temperature at which the shifted hysteresis loop effect appears. The magnet which results has one easy direction of magnetization.

In order to obtain optimum properties, the field should be maintained down to the lowest temperature to which the body is cooled. It is felt that the present magnets, as processed, acquire their unique behavior by virtue of ferromagnetic and antiferromagnetic regions present

within the body. The coupling effect between the ferromagnetic and the antiferromagnetic regions causes the one easy direction of magnetization. Therefore, during cooling of the body, it is essential that it be subjected to a magnetic field, one on the order of 5,000 oersteds normally being sufficient to properly align the antiferromagnetic as well as the ferromagnetic moments in any of the alloys. Of course, lesser fields can be used in some cases and still obtain maximum alignment of the magnetic moments within the magnet. Although the magnetic field need only be applied from just above that temperature in which the shifted loop effect begins, as a matter of expedience, it is normally easier to apply the field continuously during the entire cooling treatment.

15 The effect of cooling the body from room temperature to below the critical temperature without using a magnetic field can be seen by referring to the loop 20 of FIGURE 4 of the drawings. This loop was obtained from the same material used to obtain curve 15 in FIGURE 2, the difference resulting from the absence of an applied magnetic field during cooling. The symmetry of the loop with respect to the origin clearly indicates that the magnetic field is necessary during cooling to obtain the preferred direction of magnetization in the magnets.

20 25 Although the present invention has been described in connection with preferred embodiments, it is to be understood that modifications and variations may be restored to without departing from the spirit and scope of the invention, as those skilled in the art will readily understand. Such modifications and variations are considered to be within the purview and scope of the invention and the appended claims.

What I claim as new and desire to secured by Letters Patent of the United States is:

35 1. A magnet having one easy direction of magnetization, said magnet being composed of magnetically coupled ferromagnetic and antiferromagnetic regions and compositionally consisting of a solid solution alloy which has at least partial atomic disorder and consists of from about 5 to 30 atomic percent manganese, balance substantially all a metal selected from the group consisting of copper, silver, and gold.

40 2. A magnet as defined in claim 1 wherein said solid solution alloy consists essentially of from about 5 to 30 atomic percent manganese, balance substantially all copper.

45 3. A magnet as defined in claim 1 wherein said solid solution alloy consists essentially of from about 10 to 25 atomic percent manganese, balance substantially all silver.

50 4. A magnet as defined in claim 1 wherein said solid solution alloy consists essentially of from about 10 to 25 atomic percent manganese, balance substantially all gold.

## References Cited in the file of this patent

## UNITED STATES PATENTS

- |           |                   |               |
|-----------|-------------------|---------------|
| 2,141,113 | Peterson          | Dec. 20, 1938 |
| 2,161,253 | Hensel et al.     | June 6, 1939  |
| 2,161,574 | Hensel et al.     | June 6, 1939  |
| 2,298,261 | Mittendorf et al. | Oct. 6, 1942  |
| 2,466,202 | Brenner           | Apr. 5, 1949  |
| 2,961,360 | Kouvel et al.     | Nov. 22, 1960 |